

T. M. HART.

ROAD AND PROCESS OF MAKING THE SAME.

APPLICATION FILED JAN. 14, 1910.

1,158,418.

Patented Oct. 26, 1915.



WITNESSES:

Jedediah Blay  
Barbara Abby

INVENTOR

THOMAS M. HART

BY  
Henry S. Blackmore.  
ATTORNEY

# UNITED STATES PATENT OFFICE.

THOMAS M. HART, OF NEW YORK, N. Y., ASSIGNOR TO PEREZ M. STEWART, TRUSTEE,  
OF NEW YORK, N. Y.

## ROAD AND PROCESS OF MAKING THE SAME.

1,158,418.

Specification of Letters Patent.

Patented Oct. 26, 1915.

Application filed January 14, 1910. Serial No. 538,043.

*To all whom it may concern:*

Be it known that I, THOMAS M. HART, a citizen of the United States, residing in the borough of the Bronx, city of New York, 5 in the county of New York and State of New York, have invented certain new and useful Improvements in Roads and Processes of Making the Same, of which the following is a specification, reference being had 10 to the accompanying drawings.

This invention relates to roads and methods of constructing the same; and an object of this invention is to provide a road which will contain a minimum of void spaces and 15 which will withstand the severe shocks to which roads are now subjected by motor-vehicular traffic.

It has been conclusively demonstrated that the action of the moving wheels of motor vehicles on roads of present-day construction is to tear up and reduce to a loose dust the covering of the road which is designed to prevent the entrance of rain and snow and other disintegrating elements; and 25 this loose dust is further displaced by the air-currents created by the rapidly-moving motor-vehicles themselves. The entrance of the disintegrating elements having occurred, the larger stones which form the lower 30 strata of the road become loosened and the road rapidly deteriorates.

In the drawings illustrating the principle of my invention and the best mode now known to me of applying that principle, 35 Figure 1 is a section of a road built according to my new method and designed for heavy traffic; Fig. 2 is a section of a road built according to my new method and designed for light traffic; and Figs. 3, 4 and 40 5 are sections of modified forms of road construction designed for light traffic and built according to my new method.

In carrying out my invention, the natural base *a* of earth or clay is thoroughly rolled. 45 If the road is to be subjected to the heaviest traffic of today, a layer *b* of concrete is laid in which the largest pieces of stone will be about one inch in diameter. This layer of concrete will be tamped or rammed and will 50 be about five inches in depth or thickness. Over the top of this layer *b* of solid concrete will be laid a layer *c* of cement mortar

of a thickness of about one-half inch. The top stratum or layer *d* is made up of a series of courses or thicknesses of broken 55 stone bound together with bituminous or asphaltic material, to which alum may be added. The size of the pieces of broken stone will vary, the size used in the lowermost course being about one inch in diameter. From the lowermost course to the uppermost, the size of the stone will gradually decrease, until at the top stone dust or the finest product of the crusher will be used. In building the top layer *d* the broken stone 60 forming each course is spread and over this course is poured molten asphalt, and over the molten asphalt may be thrown powdered alum, which asphalt produces a water-repellent and protective member of the composite layers of the road-forming body combination and being substantially free from silicious ingredients, provides a top coat which is less slippery in wet or frosty weather than when it contains foreign silicious ingredients which tend to break or 65 destroy its inherent continuity and retard its natural resiliency and expansive and contractive properties under varying conditions of temperature and atmospheric pressure. The aluminium sulfate containing ingredient of the asphalt, such as alum, when present, has the tendency to cause or produce a thorough amalgamation of the asphalt by abstracting water of emulsification 70 and fixing the same as aluminous water of crystallization, and at the same time producing a resistant finish to the surface of the asphalt whereby friction is produced by the natural adherence to iron and steel, 75 such as horse shoes, tires, etc., when brought in contact therewith, which is not attained in cases where asphalt contains sand, stone, or other crystallized silicious substance 80 which has a natural attracting and retaining affinity for water, on and to the surface and in contact with such mixture, and a corresponding anchorage for ice and frost when contacting with or resting upon its surface. The water-repellent action of the 85 free and unsilicious asphalt prevents the union or retaining of water thereon or anchorage of ice thereto. The course is then 90 most thoroughly rolled or ironed, until 95

each and every stone in the course is rigidly fixed in place and the interstices between the stones are completely filled. In no event is a greater percentage of void spaces than 5 ten per cent. (10%) allowable throughout this upper layer  $d$ . The latter is built up, course by course, the same care being exercised to see that every course or thickness is thoroughly ironed or pressed and that no 10 void spaces are left; but that, on the contrary thereof, the interstices between the pieces of stone are filled by the bituminous matrix, so that disintegrating elements cannot enter or find lodgment whereby to break 15 down the solidity of the layer  $d$ , the depth or thickness of which will be about three inches.

In Figs 2 to 5, both inclusive, are shown sections of roads built according to my new 20 method and designed and adapted for light traffic. In Fig. 2 is shown a section of a road in which a layer  $e$  of burned clay broken into bits is used. This layer  $e$  is placed after the natural base of earth or 25 clay  $a$  has been thoroughly rolled and prepared to receive it. Over the stratum of burned clay is laid the top stratum  $d$  of asphaltic mixture as hereinbefore described. The method of building up this layer  $d$ , 30 course by course, is the same as that pursued in making the road shown in section in Fig. 1. The road shown in section in Fig. 3 differs from that shown in Fig. 2 in only 35 the substitution of a layer  $f$  of river silt for the layer  $e$  of broken bits of burned clay, while in the road illustrated in Fig. 4 a layer of gravel  $g$  is used instead of the burned clay or river silt. In the road shown in Fig. 5 the layer  $d$  of asphaltic 40 mixture is laid directly upon the natural base or bottom  $a$ .

The term "non-silicious" employed in the present specification and claims is intended 45 to imply and does imply an asphalt of commercial or other character *per se*, in contradistinction to and from a concrete mixture of asphalt with sand or other silicious ingredient to a degree which would affect the 50 resilient or water-repelling properties of the asphalt as such.

The substance capable of dehydrating, 55 withdrawing, abstracting, or fixing the water of emulsion in or from the asphalt and converting it into an asphalt non-repellent, such as solid water or crystallization in case of alum and similarly acting sulfates or substances, provides a means for producing and produces a thorough amalgamation or 60 union of the asphalt resulting in a solid and substantially compact, voidless, and tenacious asphaltic material. The alum or similar chemical dehydrating substance removes the water of emulsion by combining or uniting with the same and converting it into

solid water of crystallization, thereby chemically dehydrating the material by contact, thus avoiding the difficulty experienced in dehydrating asphalt by the action of heat, as employed hitherto, and producing a product of greater tenacity, resilience, and 70 utility.

The term "alum" employed in the specification and claims is intended to imply and does imply alum as such of anhydrous character or of sub-hydrous or hydrous crystalline nature, such as would be formed by the dehydration of asphalt by hygroscopic alum when associated with hydrous asphalt. 75

I claim:

1. A road or pathway comprising a composite composition bonded together by a bituminous material associated with a substance capable of converting contained water into solid water of combination. 80

2. A road or pathway comprising a composite composition bonded together by a bituminous material associated with a substance capable of converting water of emulsification into solid water of crystallization. 85

3. A road or pathway comprising a composite composition bonded together by a bituminous material associated with a metal sulfate capable of converting water of emulsification into solid water of crystallization. 90

4. A road or pathway comprising a composite composition bonded together by a bituminous material containing aluminium sulfate capable of converting water of emulsification into solid water of crystallization. 95

5. A road or pathway comprising a composite composition bonded together by a bituminous material containing alum capable of converting water of emulsification into solid water of crystallization. 100

6. The process of making a road or pathway which comprises associating the road or path body ingredients with asphalt containing a substance capable of converting water of emulsification into solid water of crystallization. 105

7. The process of making a road or pathway which comprises associating the road or path body ingredients with asphalt containing a metal sulfate capable of converting water of emulsification into solid water of crystallization. 110

8. The process of making a road or pathway which comprises associating the road or path body ingredients with asphalt containing aluminum sulfate capable of converting water of emulsification into solid water of crystallization. 115

9. The process of making a road or pathway which comprises associating the road or path body ingredients with asphalt containing alum capable of converting water of emulsification into solid water of crystallization. 120

10. The process of making a road or pathway which comprises associating the road or path body ingredients with asphalt containing a substance capable of converting 5 contained water into solid water of combination.

In testimony whereof I hereunto set my

hand at New York city, N. Y., this eighth day of January, A. D. 1910, in the presence of the two undersigned witnesses.

THOMAS M. HART.

Witnesses:

JOHN POPP,  
SAM'L BELL THOMAS.